

**1****3,709,803**

**METHOD OF TREATING METAL ARTICLES**  
Graham L. Gulick, 4559 N. Hamlin, Chicago, Ill. 60625  
No Drawing. Continuation-in-part of application Ser. No. 833,720, June 16, 1969. This application Feb. 1, 1972, Ser. No. 222,656  
Int. Cl. C23b 1/00, 3/06

U.S. Cl. 204—140

11 Claims

**ABSTRACT OF THE DISCLOSURE**

A method of toughening high speed steels and carbon steel forming and cutting tools or the like comprising immersing a steel object in an aqueous treating bath which includes a cyanide salt, an alkali metal hydroxide, a sequestering agent for ferric ions at high pH, and, using the article as one electrode, passing an alternating current through said article and said bath at a potential of about 2.5 volts and a rate of about 1.75 amperes per square inch of surface of the article for a period of about one minute or less at a temperature slightly above ambient temperature. Metals so treated also display other described advantageous properties.

**BACKGROUND OF THE INVENTION**

This application is a continuation-in-part of application Ser. No. 833,720, filed June 16, 1969 and now abandoned.

The present invention is directed generally to methods of metal treatment, and in particular, to a method of altering the brittleness-toughness characteristics of metal articles, particularly carbon and high speed steel cutting and forming tools and the like, to impart greatly improved toughness thereto.

It is well known that there are a number of thermal methods adapted to be used in hardening of carbon steel, such as heat treating and the like. Once an article such as a drill bit, cutting tool or the like has been properly heat treated, it is sufficiently hard for use, but tools treated in this manner and made from carbon or high speed steel would be more desirable if they were of increased toughness, that is, if the life of such tools could be increased or if the cutting rates or speeds thereof could be increased, or both. Thus, toughness, which qualitatively may be said to be somewhat the opposite of brittleness, is not readily measured directly, but is manifested by the ability of the cutting tool or the like to remain sharp, to be able to tolerate increased speed of metal removal, to resist damage from interrupted cutting operations, and to undergo smaller temperature rise than a less tough tool under comparable conditions.

The present invention therefore relates to a toughening treatment in which a low voltage alternating electrical current is passed through an article to be treated in the presence of a suitable electrolyte, resulting in treated metal articles, such as drill bits and the like, having vastly improved toughness.

In view of the fact that high speed cutting tools would be much more desirable if of increased toughness, and in view of the need for a post treatment for heat treated articles to provide cutting tools and the like of increased toughness, it is an object of the invention to provide a novel treatment method for toughening ferrous metal articles.

Another object is to provide a method in which an alternating current is impressed upon an article to be treated, using the article as an electrode, and subjecting the article to carefully controlled current flow while the article is immersed in a chemical treating bath.

Another object is to provide a treating method which includes passing an alternating current through a ferrous

**2**

metal article to be treated in the presence of a reducing solution under controlled conditions.

Another object of the invention is to provide a method of altering the toughness/brittleness ratio of a metal article without erosion of the metal, change in the surface finish, or change of dimensions of the treated article, that is, a method of imparting greater toughness and less brittleness to a metal article having a given hardness.

Still another object of the invention is to provide a method of treating the entire body of a metal article while exposing the surface to controlled chemical and electrical conditions.

A still further object of the invention is to provide a method of treating articles under milder conditions than those employed to descale or remove rust from such articles.

Still another object is to provide a treating method utilizing a voltage substantially lower than that used in methods for surface cleaning articles, which prior art methods serve to bring about an effect in the articles which is opposite the effect brought about by the method of the invention.

A still further object is to provide a method of providing tools, such as drill bits, forming tools, shears, thread forming rollers, and the like having increased toughness as manifested by longer life, the ability to perform a faster cutting operation and characterized by less temperature rise than untreated counterparts thereof.

Another object is to provide a method for treating a metal article so that the article, when used as a transformer core or the like, undergoes smaller temperature rises in use than like untreated articles under the same conditions.

The present invention achieves these objects and others which are inherent therein by immersing an article to be treated in an aqueous solution including a cyanide salt, an alkali metal hydroxide, a ferric ion chelating agent, and, using the article to be treated as one electrode, passing a current through the article and the bath under carefully controlled conditions of current density and at a potential of about 2 to 3 volts. The manner in which the invention is carried out will become more clear when reference is made to the accompanying detailed description of the preferred embodiments set forth by way of example, and to the appended claims.

The invention will now be described with reference to several such preferred embodiments, which serve to illustrate typical methods of practicing the invention.

**Example 1**

Initially the work to be treated, such as a drill bit or like cutting tool, is chemically cleaned with suitable solvents or otherwise by known methods to remove grease, oil, or other contaminating films. Care is taken to avoid touching the work with the fingers after cleaning thereof. In the event the articles desired to be treated are rusty or scaly, the rust or scale must be removed therefrom prior to cleaning as set forth above.

An electrolytic solution is then prepared according to the following formula:

Sodium cyanide—73.5 grams (1.5 moles)  
Sodium hydroxide—40.0 grams (1.0 moles)  
"Seqlene ES-50"—200 ml.  
Water to make one liter

The "Seqlene ES-50" is a 50% aqueous solution of the alpha and beta isomers of sodium glucoheptantate, made by Pfanziehl Laboratories, Waukegan, Ill., and is a chelating agent for ferric iron ions which is effective at high pH. The bath is placed in a glass liner or otherwise electrically insulated tank adapted to prevent stray currents, and heated to 40° C. with agitation. Preferably,

tank electrodes are 24 gauge perforated stainless steel (Type 304) sheets, and the surface area thereof is larger than that of the largest surface area of the work about to be undertaken.

A step down transformer is provided, such as a "Variac," and 60 cycle, 110 volt alternating current is supplied to the primary thereof, with the secondary being variable so as to provide from 0 to 5 volts (root mean square) across the secondary of the transformer. One terminal of the secondary is connected to the tank electrodes, through a suitable large ammeter, which is preferably and ordinarily an ammeter of the type reading the root mean square current values rather than peak current values (root mean square values being those referred to throughout this description). The other terminal of the secondary is connected to a conductive article holder clip for supporting the work in a completely immersed position in the bath. Appropriate calculations and adjustments are made to provide an operating potential of 2.5 volts and a current density of 1.75 amperes per square inch of work area, such current measurement being the root mean square current value rather than peak current value. Preferably, the work is disposed between the two tank electrodes, which are preferably held in a vertical position with their major surfaces in planes parallel to each other. The current is allowed to flow for 40 seconds at the 40° C. temperature, while the 1.75 ampere per square inch current density is maintained. Thereafter, the drill bit or the like is removed and is ready for use without further treatment.

In the case of drill bits treated according to the above set forth example and used to drill copper-epoxy-glass laminate used in the construction of printed electrical circuit boards, for example, the average life of such units was about 75% of the life of solid carbide drill bits costing ten times as much as the high speed steel drill bits treated for toughness according to the invention. A drill bit prepared in this manner has excellent resistance to shock, and thereby is particularly advantageous for use where shock conditions are present and tend to damage, even extremely hard drill bits, such as carbide bits. As an example, an operation involving interrupted cuts creates severe shock, and damages or rapidly destroys such bits or cutting tools which, although very hard, are relatively brittle.

#### Example 2

A treatment of the tool bit was carried out according to the method of Example 1, except that the current density was about 2.5 amperes per square inch of surface area of the tool. This current density was operative to produce a toughened tool in some cases, but in other cases, appeared to cause slight softening of metal, and on the average was not nearly as effective as the 1.75 ampere per square inch current density of Example 1.

#### Example 3

Treatment of a drill bit was carried out according to the method of Example 1 except that the current density was held at from about 1.0 to 1.25 amperes per square inch. In this example, the cyanide salt was also present in the ratio of 1.5 moles per liter, but was a potassium cyanide salt rather than sodium cyanide, and the alkali metal hydroxide was potassium hydroxide, which was present in a concentration of 1.0 moles per liter. On the average, this current density was not sufficient to produce a significantly improved tool, although in some cases, an improved tool could be produced by this method.

As a result of considering Examples 2 and 3, it was determined that an optimum current density range is from about 1.25 amperes per square inch or more to about 2.25 amperes per square inch or less, and that 1.75 amperes per square inch is preferred. The preferred voltage was 2.5. While voltages of about 2 volts to 3 volts were satisfactory, voltages of higher values, such as 5 volts or more, produced unsatisfactory articles having undesirably soft

and/or brittle surfaces rather than surfaces of increased toughness.

#### Example 4

5 A treating bath was prepared using only about 0.5 mole per liter (24.5 grams per liter) of sodium cyanide, 0.3 mole (12 grams per liter) of sodium hydroxide, and about 50 ml. of the "Seqlene ES-50" (50% solution) with a current density of the order of 1.75 ampere per square inch and a 2.5 volt potential, for a time of between 35 10 and 45 seconds. Excellent results were also obtained when a tool was treated with this method. A tool was also successfully treated using potassium cyanide and potassium hydroxide in the above set forth molar concentrations.

#### Example 5

Treatment of a tool bit was again carried out under the same conditions as those referred to in Example 1, except that approximately 4.5 moles per liter (220 grams per liter) of sodium cyanide, about 3 moles per liter (120 grams per liter) of sodium hydroxide, and about 250 ml. of "Seqlene ES-50" were used. At a current density of 1.75 ampere per square inch of work, a temperature of 40° C. and a 40 second cycle time, good results were obtained.

25 Thus, considering Examples 4 and 5, it is apparent that the concentrations of the cyanide, the alkali metal hydroxide, and the ferric ion chelating agent are not particularly critical, although the preferred concentrations are those set forth in Example 1.

#### Example 6

A treating operation similar to that described in connection with Example 1 was carried out, except that the chelating agent used was triethanolamine. The triethanolamine performs satisfactorily, but is more costly and not always as effective as the "Seqlene ES-50" reagent, and accordingly, is not preferred.

In connection with the methods described in the above examples, and other similar methods, it was also determined that temperatures below 40° C. were operable, although temperatures in the 40° C. range tend to give somewhat increased speed of the treating cycle time than lower temperatures.

45 It is also known to those skilled in the art that relatively high temperatures cause decomposition of the cyanide reagent, and accordingly, such high temperatures are preferably to be avoided. The 40 second cycle time, plus or minus about 4 seconds, is preferred, although cutting aid forming tools have been improved by the 50 process of the invention using time periods falling significantly outside this range.

55 It is not known with certainty why the present invention produces such remarkable results in increased tool toughness and longevity of sharpened tool edges as well as tools capable of higher cutting rates and lower operating tool temperatures, as compared to untreated tools having the same speeds and cutting rates; however, it is considered possible that the mechanism of hardening a carbon steel includes the adsorption of 60 atomic hydrogen at a number of sites on the surface of carbon particles which are located at the grain boundaries, and that this adsorption can be controlled by the method of the present invention. It is thought that these carbon particles may adsorb hydrogen upon 65 their surface, and under ideal conditions, when the correct quantity of hydrogen is adsorbed on the surface of the particle, it is difficult for these metal grains to slip past one another under applied stress, and the hardness of the metal is greatly increased. However, the number of sites at which carbon may adsorb hydrogen are thought to be varied in number and character. Thus, the carbon particles may contain a number of sites, considered to be primary sites, wherein hydrogen is adsorbed with a release of considerable energy and where such hydrogen is therefore strongly held. Even when all of

these sites are filled, it is believed that additional hydrogen may be attracted to additional sites, which may be considered secondary sites, of relatively more indefinite number and qualitatively characterized by less energy of adsorption, and whereto hydrogen is consequently less strongly attracted.

It is also thought possible that the mobility of atomic hydrogen within the metal during ordinary tempering or heat treating is sufficient so that hydrogen is rapidly attracted to grain boundary carbon during periods of proper metal temperature, and that the hydrogen mobility and speed of adsorption are so great that additional or secondary hydrogen adsorption may take place at secondary sites rapidly and in a manner which, undesirably, is difficult to control. Excessive or secondary adsorbed hydrogen is thought to cause a forcing apart or rift of adjacent grains, and with inter-granular cohesion of the metal being greatly reduced at such points, the metal remains hard but is undesirably brittle. It is believed possible that maximum hardness occurs when all so called primary adsorption sites are filled, but that brittleness is significantly increased as secondary adsorption takes place, whereas when sufficient hydrogen to fill all primary sites only is available, maximum toughness is obtained.

In keeping with the possible explanation set forth above, it will be understood that the thermal mobility of hydrogen may be considered, for practical purposes, to have a threshold or minimum critical temperature. In such a case, where the mobility is brought about by increased temperature, as a practical matter, it is not possible to obtain sufficiently exact hydrogen mobility so that hydrogen will be entirely adsorbed at the primary sites, but not at all at secondary sites, the ideal condition at which the metal achieves maximum toughness. Therefore, the method of the present invention is one in which this mobility may be controlled by providing proper electro-chemical conditions, rather than by thermal means, and one in which means are provided for the excess hydrogen thus mobilized to escape.

It is thought possible that the present invention provides a low temperature method of restoring or increasing the mobility of this adsorbed atomic hydrogen and by providing a phase boundary at the metal surface across which excess adsorbed hydrogen may escape, so that processing may take place without increasing the temperature beyond ambient temperature, or to the orders of temperature at which thermal mobility of adsorbed or adsorbable hydrogen becomes a significant factor. It is therefore thought possible that with the general mobility of all adsorbed hydrogen reduced by reason of reduced ambient temperature, the release rate of hydrogen adsorbed at secondary sites is therefore subject to accurate control so that the hardness of the parent metal need not be altered, and yet the toughness thereof can be significantly increased.

In this connection, it is believed that the passage of alternating current through a magnetically influenced or magnetically affected metal may stress the crystal structure of the metal sufficiently to permit the desired limited mobility of weakly adsorbed hydrogen held on the carbon particles, particularly in the presence of a suitable electrolyte in contact with the metal surface to provide mobility and escape of excess hydrogen.

It is believed that by using a lower potential, of 2 to 3 volts for example, than that previously used for the purpose of descaling ferrous metal articles, desirably mild conditions are used to bring about the controlled release of secondary hydrogen. Thus, prior art methods using higher voltage might be thought of as analogous to prior art methods involving high temperature, that is, the more severe conditions cause loss of control, and relatively indiscriminate loss of primary and secondary hydrogen. The present method, however, uses much lower voltage and consequently toughens the metal without

causing surface embrittlement characteristic of prior art descaling methods.

The electrolyte appears to be able to allow limited amount of hydrogen to be released from the metal across the phase boundary and the hydrogen may then be released from the solution in detectable quantities. At any rate, however, neither the exact behavior of the hydrogen, within the metal or in the solution, nor the existence or the operation of the above postulated mechanism forms an essential part of the present invention, and is not intended to limit the scope thereof.

Referring again to the treated articles and method, the treating bath has been discovered to have an extremely long service life requiring only infrequent additions thereto. After long use, crystals of sodium ferrocyanide may be found on the bottom of the tank, possibly resulting from the reaction of iron and sodium cyanide in the presence of water to yield sodium ferrocyanide, sodium hydroxide and hydrogen in the presence of, or under the influence of alternating current.

A principal advantage of the invention is that the treated articles such as stock high speed steel cutting tools, forming tools and the like merely taken from the shelf and treated as set forth above will produce 2 to 10 times more work pieces before resharpening is necessary than will their otherwise identical but untreated counterparts. Resharpening these tools by conventional methods does not cause loss of the beneficial advantages of increased toughness achieved by treatment as set forth above.

Although tools treated according to the present invention give excellent results when used on any work which is less hard than the tool itself, best results have been obtained on non-ferrous metals and alloys, on non-magnetic ferrous alloys, and on non-metals among which are the reinforced or filled plastics referred to above.

It is also discovered that increasing the tool working clearances over and above those suggested by cutting tool manufacturers gave significantly further improved results, thinner cross sections being required to support the cutting edge of the cutting tool. Experimental measurements have thus far indicated that superior performance results even without increased clearance, but that tools treated according to the above method and with greater clearance display outstanding results.

A still further advantage of the treating method of the invention is that tools thus treated also display greatly increased resistance to atmospheric corrosion.

In addition to drill bits which were illustrated as being typical tools upon which the present invention may be practiced with advantage, end mills, ordinary kitchen knives, shears, including those used on paper, those used by barbers, for example, and hand files, for example may be advantageously treated by this method. In the case of hand files, it has been noted, particularly when using them on softer metals such as aluminum or the like, clogging of the files has been significantly reduced or eliminated, indicating that the soft metals do not tend to cling to or remain attached to the surface of the cutting metal, and this results in significantly improved performance by way of increased production rates, and greater convenience in use of the files.

Another area in which the present invention demonstrated unexpectedly favorable results was in the field of treating piston rings used for internal combustion engines.

Piston rings treated as set forth above in Example 1 were used in a gasoline engine, and, for reasons which are not understood fully, demonstrated extremely long life in use as compared with otherwise similar but untreated piston rings.

Other articles which demonstrated unexpected properties when treated according to the method of the invention were the laminations from electrical transformer cores. For example, the core of an electrical transformer was disassembled and the individual laminations treated according to the method of Example 1. When the lamination

tions were reassembled and placed in the same transformer, it was noted that under relatively large load, a much smaller temperature rise than previously noted was experienced. Also, when lighter loads were impressed on the transformer, no temperature rise was detectable, under the same load, with the treated core, whereas the untreated transformer core underwent a noticeable although unobjectionable temperature rise. Accordingly, a transformer with a treated core had a larger useful load capacity or rating than a transformer with an untreated core.

It will thus be seen that the present invention provides a novel tool treating method having a number of advantages and characteristics including those herein pointed out and others which are inherent in the invention.

I claim:

1. A method of treating a ferrous metal article to increase the toughness thereof comprising immersing said article in an electrolyte comprising an aqueous solution of an alkali metal hydroxide, a soluble cyanide salt, a chelating agent for ferric ions at high pH, and passing an alternating electrical current through said article to another electrode immersed in said solution at a potential of from about two to about three volts and at a current density of from about 1.25 to about 2.50 amperes per square inch of article to be treated.

2. A method as defined in claim 1 in which said cyanide salt is selected from the group consisting of sodium cyanide and potassium cyanide.

3. A method as defined in claim 1 in which said alkali metal hydroxide is selected from the class consisting of sodium hydroxide and potassium hydroxide.

4. A method as defined in claim 1 in which said chelating agent is sodium glucoheptanate.

5. A method as defined in claim 1 in which said period during which said article is from about 20 seconds to 35 about one minute.

6. A method as defined in claim 1 in which said cyanide salt is present in an amount of from about 1.0 to about 2.0 moles per liter and in which said alkali metal hydroxide is present in a quantity of about 0.75 to about 1.5 moles per liter of solution.

7. A method as defined in claim 6 in which said che-

lating agent is present in an amount of from about 25 to about 250 grams of active ingredient per liter of treating solution.

5 8. A method as defined in claim 1 in which said treated article comprises a cutting or forming tool.

9. A method as defined in claim 1 in which said chelating agent is triethanolamine.

10 10. A method as defined in claim 1 in which said cyanide salt is present in an amount of from about 0.45 to about 4.5 moles per liter and in which said alkali metal hydroxide is present in an amount of from about 0.3 to about 3.0 moles per liter of solution.

11 11. A method of treating a cutting tool made from a ferrous metal comprising immersing said article in a bath containing an aqueous solution of about 1.5 moles per liter of a soluble cyanide salt, about 1 mole per liter of an alkali metal hydroxide, about 100 to 200 grams per liter of a ferric ion chelating agent effective at high pH, and, using said article as one electrode, passing a 60 cycle per second alternating current through said bath at a potential of about 2.5 volts and a root mean square current density of about 1.75 amperes per square inch of surface area of said article, for about 40 seconds.

25

#### References Cited

##### UNITED STATES PATENTS

|           |         |                 |       |         |
|-----------|---------|-----------------|-------|---------|
| 2,057,274 | 10/1936 | Mayhew          | ----- | 204—140 |
| 3,420,760 | 1/1969  | Freedman et al. | ----- | 204—145 |
| 3,207,683 | 9/1965  | Hermann         | ----- | 204—141 |

##### FOREIGN PATENTS

|           |         |                |
|-----------|---------|----------------|
| 200,740   | 1/1939  | France.        |
| 663,217   | 12/1951 | Great Britain. |
| 1,269,443 | 5/1968  | Germany.       |

JOHN H. MACK, Primary Examiner

T. TUFARIELLO, Assistant Examiner

40 U.S. CL. X.R.

204—140.5